

Jan. 6, 1959

W. M. MacNEVIN

2,867,546

GAS PLATING OF ALUMINUM USING ALUMINUM TRIISOBUTYL

Filed Feb. 8, 1956



Fig. 1



Fig. 2



INVENTOR

WILLIAM M. MacNEVIN

BY

*Taulmin & Taulmin*

ATTORNEYS

1

2,867,546

## GAS PLATING OF ALUMINUM USING ALUMINUM TRIISOBUTYL

William M. MacNevin, Columbus, Ohio, assignor to The Commonwealth Engineering Company of Ohio, Dayton, Ohio, a corporation of Ohio

Application February 8, 1956, Serial No. 564,180

10 Claims. (Cl. 117—107)

This invention relates to gas plating of aluminum and to composite bodies produced thereby.

The problem of producing a coating of aluminum by volatilization of the metal and condensing the same onto a surface to be plated has failed of solution because the high temperatures involved in such a process made success impossible. A temperature of 1800° C. (3272° F.) is required to form aluminum metal vapor. The difficulties involved in handling such high temperature metal vapor, which has an avid tendency to react with oxygen, hydrogen or other elements presented an insoluble problem.

In accordance with the discovery of the present invention, gas plating of this light metal is carried out at relatively low temperatures and pressures by the use of a heat-decomposable gaseous aluminum alkyl, e. g., triisobutyl aluminum. The material to be plated with aluminum metal is placed in a chamber and the air is replaced with an inert gas such as nitrogen.

While thus protecting the article to be plated or aluminized, triisobutyl aluminum is introduced into the chamber, preferably utilizing an inert carrier gas such as nitrogen. Deposition of the aluminum metal is accomplished by heating the base material to a temperature sufficient to decompose the aluminum triisobutyl when brought in contact with the heated article, thus releasing aluminum metal which is plated onto the surface of the article.

The present invention makes it possible to deposit aluminum on the surfaces of various materials, and such as will withstand the temperature used to bring about decomposition of the gaseous aluminum alkyl. Plating of the light metal may be made on various metal surfaces, e. g., steel, iron, copper, magnesium, or metal alloys as well as non-metal materials, e. g., glass, molded plastics, wood, paper and the like.

Due to the nascent physical state of the aluminum metal, the same being deposited as it is liberated from the gaseous compound, a metal film of one molecule thickness is provided initially which may be further increased as desired. Thus a tenacious metal layer of aluminum is formed in the surface pores of the base material on which the metal is deposited.

The process of the invention permits rapid deposition of light metals, e. g., aluminum at relatively low temperatures and pressures as compared to prior processes utilizing volatilized metals.

In gas plating metal surfaces, for example the metal, after being thoroughly cleaned of foreign matter, is subjected to gas plating utilizing a suitable organo-metallic compound of aluminum and which compound is heat-decomposable at temperatures substantially below the vaporization point of the light metal. The decomposition or disassociation of the gaseous metal compound is made to take place in an atmosphere which is inert to the nascent metal, being especially free of oxygen, hydrogen and water. An atmosphere in the plating chamber of dry nitrogen gas has been found suitable. This inert gas

2

also may be used as a carrier and protecting blanket for the aluminum alkyl compound. Other gases which are inert and free of oxygen and moisture may be used in place of nitrogen, such as helium, argon, etc.

5 In carrying out the aluminum metal plating in accordance with the preferred practice of this invention, the material to be plated is placed in a closed chamber or container having an inlet and outlet opening. Thereafter the air and water vapor are displaced by forcing dry 10 nitrogen through the chamber under sufficient pressure to displace the air. Aluminum triisobutyl, which is contained in a bottle or suitable container filled with nitrogen under pressure is then introduced into the plating chamber.

15 To bring about decomposition of the aluminum alkyl after the same is introduced into the plating chamber, suitable heating means is provided to heat the material to be plated to a temperature high enough to cause the gaseous aluminum triisobutyl compound to decompose 20 and aluminum metal deposited on the surface of the material. Heating of the material may be accomplished in any suitable manner. Where the plating chamber is made of glass or plastic material which will transmit infra-red rays, heating may be effected by the use of infra-red lamps. Electrical resistance heating means also 25 may be employed if desired. To this end Nichrome resistance wires or ribbons may be wound around the plating chamber enclosed in asbestos felt, or the like, and connected to a source of electricity to heat the chamber and material or article therein to bring about decomposition of the aluminum alkyl gaseous compound.

30 Aluminum triisobutyl preferably is conducted into the plating chamber utilizing nitrogen as a carrier gas and the flow rate is controlled whereby the air is displaced 35 and prevented from flowing back into the plating chamber during operation of the process. For this purpose, a blower or pump may be connected to the system and operated to control the flow of gases therethrough. Gas plating of base material with aluminum may thus be accomplished in a matter of seconds. Further, any aluminum alkyl compound which is not decomposed initially 40 may be recovered and recirculated back through the plating system, the same being enriched with fresh aluminum alkyl from time to time as required.

45 The surface of the material to be plated with aluminum is initially cleaned of foreign matter and dried to remove moisture. Manual or chemical cleaning means or a suitable combination thereof may be employed for this purpose. Sandblasting, wire brushing or the like are 50 suitable methods to remove solid foreign matter from metal surfaces. Where the surface is to be de-greased and cleaned, the same may be washed with petroleum solvent, such as xylol, toluol or the like, and all traces of moisture are removed by heating the material at 250 to 300° C. for a time sufficient to drive off any residual 55 moisture.

After the article has been cleaned thoroughly and freed of all moisture and rendered chemically clean, the same is introduced into the nitrogen filled plating chamber and heated as described. While the article is heated 60 in the plating chamber under an atmosphere of nitrogen, aluminum triisobutyl is introduced and the gaseous aluminum alkyl brought in contact with the surface of the heated article, the temperature of the latter being high 65 enough to cause the gaseous aluminum alkyl compound coming in contact therewith to decompose or disassociate and deposit aluminum metal onto the surface of the article. After a desired thickness of aluminum deposit is obtained, the process is stopped and excess aluminum alkyl returned to storage.

70 Triisobutyl aluminum is supplied in steel pressure bottles, with brass valves. The pressure bottle which is

fitted with a rubber dam is packed to a maximum of 60% of the free volume with triisobutylaluminum liquid, and the remaining space is pressurized to a maximum of 30 pounds/sq. in. gauge with nitrogen. To remove the contents, the bottle is provided with an adapter valve and tube outlet connection to allow the internal pressure to push out the liquid when the bottle is inverted. Fittings should be opened under a blanket of nitrogen and receiving containers should be dry and previously flushed with dry nitrogen. Storage temperatures for aluminum triisobutyl are kept below 60° C. and preferably 0° to 10° C.

A suitable procedure for handling and transferring a solution (47%) of aluminum triisobutyl in normal heptane to a hypodermic syringe from storage pressure bottles was accomplished as follows.

A gas tight fume box, fitted with a trap chamber was constructed from clear plastic, e. g., Lucite. The box was provided with suitable inlet and outlet openings for receiving tubular conduit connections, the inlet being connected to a source of nitrogen gas and nitrogen pumped into the fume box to completely displace air and water vapor. To purify the nitrogen gas, it is preferably pumped through a tower containing soda lime and calcium chlorine to remove CO<sub>2</sub> and moisture prior to its introduction into the fume box. The auxiliary trap chamber of the fume box allows introduction and removal of objects from the main body of the fume box without the introduction of air.

For removing aluminum triisobutyl from the pressure bottle, a hypodermic syringe equipped with a #1, 19 gauge needle was used. After cleaning and thoroughly drying the syringe, the same was placed in the trap chamber of the fume box and the air in the syringe displaced with nitrogen by reciprocating the plunger of the syringe several times. The pressure bottle containing aluminum triisobutyl was then placed in the main chamber of the fume box, and the syringe plunger withdrawn to fill the syringe with nitrogen equal to the volume of liquid aluminum alkyl to be removed from the pressure bottle. After inserting the needle of the syringe through the rubber dam of the pressure bottle, nitrogen in the syringe was then forced into the bottle, the bottle and syringe being inverted and the plunger of the syringe slowly withdrawn to its original position to thus fill the syringe with the aluminum alkyl solution. The syringe needle was then withdrawn from the dam and the pressure bottle returned to storage, the same being preferably kept at 0° C.

Transfer of aluminum triisobutyl solution to the decomposition or plating chamber in controlled amounts for gas plating with aluminum was accomplished by expelling the desired amount of the aluminum alkyl from this syringe by working the plunger.

Apparatus suitable for carrying out the gas plating with aluminum alkyl is illustrated in the drawings, wherein—

Figure 1 illustrates an embodiment for gas plating using a horizontally arranged plating chamber; and

Figure 2 illustrates a similar apparatus wherein a vertical gas plating chamber is utilized.

Referring more particularly to the apparatus or system shown in Figure 1, nitrogen carrier gas stored in a container 10 is forced through the apparatus during plating to maintain the same free of air or oxygen. The carrier gas is oil-pumped from the storage container 10 by a pump 11 whereby the inert gas flows through conduit 12 and is discharged into the bubbler tube 13. This bubbler tube is partially filled with normal heptane, as indicated at 14, and into which the discharge end of the conduit 12 is placed. Carrier gas is led from the bubbler tube 13 by a conduit 15 and thence to a second bubbler tube 16 which comprises a side arm 17 fitted with a rubber dam 18 for receiving a needle 19 of a plunger-actuated syringe 20.

The bubbler tube 16 is heated electrically by heating

element or pad 21, and such as formed of asbestos and Nichrome resistance wire, and which surrounds the bubbler tube. The bubbler tube 16 is similarly partially filled with normal heptane 22 as in the bubbler tube 13.

Exit gas flowing from the bubbler tube 16 is discharged from the tube through a conduit 24 and into a plating tube or chamber 25. The plating chamber in this instance (consists of a hermetically sealed quartz glass tube (3/4 x 30") having an inlet 26 and an outlet 27. Conduit 24 is connected to the inlet 26 and the outlet 27 is connected through conduit 28 to a condenser bubbler tube 29 filled with heptane 30. The end closure plug 31 of the plating chamber is normally in place, as shown, but is adapted to be removed for inserting the material to be plated. A copper rod 32 constituting the material to be aluminum plated is suitably supported in the plating tube, as shown. To heat the plating chamber and copper rod to be plated, the glass plating tube 25 is made into a resistance heater by connecting the tube in an electrical circuit as across terminals 33 and 34. The resistance is made such that a steady temperature of approximately 295° C. is reached in the plating tube.

For condensing aluminum alkyl, for re-use, the bubbler tube 29 is provided with a jacket 38 into which a suitable refrigerant is circulated therethrough through the inlet and outlet conduits 35 and 36 respectively. Waste gases are discharged from the bubbler tube 29 by a conduit 37. The condenser bubbler tube is preferably maintained at a temperature of about 0° C. so that any undecomposed aluminum alkyl is condensed and recovered in the heptane.

Nitrogen carrier gas is forced through the apparatus at a rate sufficient to prevent back flow of air (oxygen) when the plating tube is opened, as when inserting material to be plated.

In the apparatus illustrated in Figure 2, a similar arrangement is used as in Figure 1, except the plating tube or chamber is disposed vertically and the inlet for nitrogen carrier gas and aluminum alkyl is disposed in the bottom of the plating chamber, as shown.

In the apparatus shown, nitrogen gas stored in container 40 under pressure is pumped, as by means of an oil-pump 41 through conduit 42 into the bubbler tube 43 and into the heptane 44 which partially fills the tube. Exit carrier gas from the bubbler tube 43 is conducted through conduit 45 to a second bubbler tube 46 which is of similar construction as bubbler tube 16, the same being partially filled with normal heptane, designated 47, and heated by an electrical heating element 48 which surrounds the tube. After flushing out air and water vapor from the apparatus, aluminum alkyl is introduced into the bubbler tube 46 by means of a syringe 59, as heretofore described. The aluminum alkyl mixes with the carrier gas and is carried along through conduit 51 to a vertically arranged plating tube 52. The plating tube in this instance is made of ordinary glass (3 x 12") and is heated by an asbestos-Nichrome ribbon electrical resistance pad 53 arranged therearound. Electrical connection to a power source is controlled to heat the plating tube, and material to be plated to a temperature such as to cause decomposition of the aluminum triisobutyl and deposition of aluminum. Material to be plated, e. g., a brass rod 55, is suitably supported in the plating tube, as by a hook 56. The exit end at the top of the plating tube 52 is connected with a conduit 57 which leads into a condenser bubbler tube 58. This bubbler tube is partially filled with normal heptane as at 59, similarly as the condenser tube 29 of Figure 1. Refrigerant is suitably circulated through the jacket 60 so as to maintain the condenser tube at a temperature of around 0° C. Exhaust gases are conducted from the bubbler tube 58 by way of conduit 61.

The following examples are illustrative but not limitative of the process of gas plating aluminum onto base materials in accordance with this invention.

## EXAMPLE I

Using the apparatus set up as illustrated in Figure 1, nitrogen is admitted to sweep out the air and the heating elements for the bubbler tubes and plating tubes are turned on to heat the same to around 295°. The syringe is charged with 5 cc. of aluminum triisobutyl heptane solution and, after allowing about 20 minutes for the apparatus to become free of air and the plating tube to reach 295° C., the plating is initiated by introducing aluminum triisobutyl into the bubbler tube and adjusting the flow of carrier gas until heavy fumes are formed in the plating tube. Deposition of aluminum begins immediately as soon as the fumes reach the hot metal in the plating tube. After the desired thickness of aluminum plate has been formed, the addition of aluminum alkyl is stopped and the remaining portion left in the syringe is returned to storage.

## EXAMPLE II

In this instance the apparatus illustrated in Figure 2 of the drawings was used. A rod of copper was placed in the plating chamber for plating the aluminum, and the plating tube heated to 300° C. Nitrogen gas was forced through the plating chamber for approximately 20 minutes to sweep out the air, thereafter a slow stream of nitrogen was permitted to flow through the gas plating chamber while aluminum triisobutyl was admitted thereto from the syringe as in Example I. The dense fumes of aluminum alkyl were decomposed and aluminum metal deposited as a uniform film onto the surface of the rod.

## EXAMPLE III

In this example gas plating of aluminum was carried out as described in Example I, using small steel strips as the material to be plated. A plating deposit of aluminum is formed on the steel to provide a composite steel-aluminum structure.

The minimum flow rate of gas is governed by whether or not the fumes of triisobutyl reach and surround the hot metal or article to be plated. If the flow rate is too slow, the fumes either condense on the walls of the connecting tubes of the apparatus or else a heavy layer of white fumes accumulates in the lower half of the tube and the base metal is covered only partially. Too rapid gas flow carries undecomposed aluminum triisobutyl out of the plating chamber, which of course, is undesirable. Also too rapid flow rate lowers the temperature inside the plating chamber and break down of the aluminum alkyl tends to occur.

The optimum rate of flow has been found to be one that will carry the aluminum alkyl into the decomposition tube or plating chamber without condensation, and which will disperse it over the whole cross section of the plating chamber so as to fill the chamber uniformly. The flow rate in each instance was maintained high enough to keep the tube filled with aluminum alkyl fumes whereby a substantially uniform even deposit of aluminum is formed on the article being plated.

The proper carrier flow rate of nitrogen in the vertical decomposition tube is slower than that used for the horizontal tube plating chamber. In the use of the vertical tube or plating chamber the white aluminum alkyl fumes gradually build up from the bottom and tend to fill the entire space. The rate of flow that need be maintained is thus adjusted whereby it is just enough to keep the vertical tube or plating chamber filled with aluminum alkyl fumes without building up of fumes in the lower portion of the tube.

The minimum temperature that will vaporize aluminum triisobutyl at a significant rate under one atmosphere pressure has been observed to be about 90° C. The density of triisobutyl aluminum at 20° C. is 0.8. At temperatures of 115° to 120° C. its rate of decomposition is relatively slow so that as a result much of the aluminum alkyl vapor remains undecomposed at this

temperature. It has been found by test runs, however, that temperatures between 275° C. and 325° C. give good decomposition of the aluminum alkyl and quality deposits of aluminum. At 350° C. the aluminum deposit on copper metal is of dark bluish color, and a clear reflecting mirror is formed on the inside of a glass tube used as a plating chamber. When the plating temperature was raised to 400° C., the mirror-like deposit formed was observed to be dark in color and not as good as where a lower temperature was used.

Triisobutyl aluminum, as supplied by the Hercules Powder Company is in liquid form. The composition as shipped consists of 60% triisobutyl aluminum:

15  $\text{Al}[\text{CH}_2-\text{CH}-(\text{CH}_3)_2]_3$ , 40% diisobutyl aluminum hydride:  $\text{Al}(\text{H})[\text{CH}_2-\text{CH}-(\text{CH}_3)_2]_2$ .

## Physical characteristics

|    | Triisobutylaluminum<br>$\text{Al}[\text{CH}_2-\text{CH}-(\text{CH}_3)_2]_3$                                                  | Diisobutylaluminum hydride<br>$\text{Al}(\text{H})[\text{CH}_2-\text{CH}-(\text{CH}_3)_2]_2$ |
|----|------------------------------------------------------------------------------------------------------------------------------|----------------------------------------------------------------------------------------------|
| 20 | Melting point 0° C.<br>Density, 20° C. 0.8.<br>Boiling point...<br>Begins to decompose when distilled above 90° C. at 1 atm. | 0.775.<br>Stable when heated to 200° C. at 1 atm.                                            |
| 25 | Boiling point 40° C. at 0.1 mm.                                                                                              | Boiling point 105° C. at 0.1 mm. Hg.                                                         |

## Chemical characteristics

30 It flames upon contact with moisture or moist air; even extremely rapidly oxidized in dry air. Reacts vigorously with compounds containing active hydrogen. Stable below 60° C.; a sample stored at 60° C. for 72 hours developed two pounds per square inch gage pressure on bringing to temperature. Pressure remained steady for the rest of the time.

35 Triisobutylaluminum can be distilled with care to keep boiling temperature below 90° C. For instance, a boiling point of 52° C. has been recorded at 0.5 mm. Hg. If small amounts of isobutylene split off, they will go over into the cold trap and the distillate will remain pure. The residual monohydride will remain in the high boiling residue.

40 The plated materials, if desired, may be subjected to an annealing heat treatment after the plating operation to stabilize the metal deposit. Such a heat treatment may consist of heating the plated article up to 400° C. for one hour.

45 The plated materials, if desired, may be subjected to an annealing heat treatment after the plating operation to stabilize the metal deposit. Such a heat treatment may consist of heating the plated article up to 400° C. for one hour.

50 The invention provides a process for plating aluminum metal directly on the surface of articles whereby there is produced a composite product comprising an outer layer of aluminum or light metal intricately and tenaciously bonded thereto.

55 The thickness of the light metal coating may be controlled by varying the time the metal bearing gas is in contact with the heated material to be plated. A coating of one molecule thickness up to one or more thousandths of an inch may be effected utilizing the process of the invention to thus provide a protective coating of aluminum on various metal surfaces or the like, the invention being especially useful to overcome corrosion problems.

60 The process further makes possible the continuous straight line production of composite products; and long length strips or sheets of material, e. g., such as used in the making of screens and the like which may be gas plated with aluminum. The invention is particularly useful in aluminizing metals where it is desired that aluminum be deposited in the pores and interstices of the base metal surface to form a substantially integral outer shell of the corrosion resistant light metal.

Preheating and drying of the article prior to gas plating preferably is carried out in an inert atmosphere such as nitrogen gas, helium and the like to prevent oxidation. Thereafter the heated and completely dry moisture free article is subjected to gas plating with gaseous aluminum triisobutyl as described.

The aluminized metal articles, as plated, are free of oxides, but upon its removal from the plating chamber and subjection to the surrounding atmosphere, an outer coating of aluminum oxide is immediately formed. This, however, does not detract from the process inasmuch as this oxide film on aluminum metal functions to protect the same as is well known.

It will be understood that while there has been described and set forth certain specific embodiments of this invention, it is not intended that the invention be thus limited thereto and it is manifest that various substitutions and changes may be made by those skilled in the art and to which the invention is readily susceptible without departing from the spirit and scope of this disclosure and as more particularly set forth in the appended claims.

What is claimed is:

1. A method of aluminum plating material which comprises establishing a source of dry inert gas free of oxygen and moisture, enclosing said material to be plated in a plating chamber filled with said inert gas, introducing aluminum triisobutyl into said plating chamber and in contact with said material, and heating said material to a temperature to cause decomposition of said aluminum triisobutyl and deposition of aluminum onto the surface of said material.

2. A method of aluminum plating material which comprises establishing a source of dry nitrogen gas free of oxygen and moisture, enclosing said material to be plated in an atmosphere of said dry nitrogen, introducing aluminum triisobutyl into said plating chamber and in contact with said material, and heating said material to a temperature to cause decomposition of said aluminum triisobutyl and deposition of aluminum onto the surface of said material.

3. A method of aluminum plating material which comprises establishing a source of dry nitrogen gas free of oxygen and moisture, enclosing said material to be plated in an atmosphere of said dry nitrogen, introducing aluminum triisobutyl into said plating chamber and in contact with said material, and heating said material to a temperature to cause decomposition of said aluminum triisobutyl and deposition of aluminum onto the surface of said material, said nitrogen gas being admixed with gaseous aluminum triisobutyl and conducted into said plating chamber and into contact with the heated material to be plated.

4. In a method of depositing aluminum on an article, the step of passing over said article vapors of aluminum triisobutyl together with an inert carrier gas free of oxygen and moisture heated to a temperature sufficient to

cause said vapors to decompose and aluminum metal to be deposited onto said article.

5. In a method of depositing aluminum on an article, the step of passing over said article vapors of aluminum triisobutyl together with an inert carrier gas free of oxygen and moisture heated to a temperature of about 295° C. and 450° C. sufficient to cause said vapors to decompose and aluminum metal to be deposited onto said article.

6. A method of aluminum plating a metallic object which comprises the steps of heating the object to a temperature of about 400° C., vaporizing aluminum triisobutyl, and contacting the heated object with the vaporized aluminum alkyl compound.

7. A method of aluminum plating a metallic object which comprises the steps of heating the object to a temperature of about 400° C., vaporizing aluminum triisobutyl with nitrogen free of oxygen and moisture at a temperature of about 300° C., and flowing the gaseous mixture of nitrogen and aluminum triisobutyl into contact with said heated object.

8. A method of plating a metallic object with aluminum which comprises the steps of heating the object to be plated in an atmosphere of dry nitrogen free of oxygen and moisture, said article being heated to a temperature sufficient to cause gaseous aluminum triisobutyl brought in contact therewith to decompose, and then contacting said heated article with said gaseous aluminum compound while enclosed in an inert atmosphere and at substantially atmospheric pressure.

9. A method of plating a metallic object with aluminum which comprises the steps of heating the object to be plated in an atmosphere of dry nitrogen free of oxygen and moisture, said article being heated to a temperature sufficient to cause gaseous aluminum triisobutyl brought in contact therewith to decompose, and then contacting said heated article while retained in a dry atmosphere of inert gas with a gaseous mixture comprising nitrogen and aluminum triisobutyl and at substantially atmospheric pressure.

10. As an article of manufacture, a gas plated product made in accordance with claim 1.

#### References Cited in the file of this patent

#### UNITED STATES PATENTS

|           |         |               |
|-----------|---------|---------------|
| 1,497,417 | Weber   | June 10, 1924 |
| 2,643,959 | Fischer | June 30, 1953 |
| 2,694,651 | Pawlky  | Nov. 16, 1954 |

#### FOREIGN PATENTS

|         |               |               |
|---------|---------------|---------------|
| 122,717 | Australia     | Nov. 21, 1946 |
| 722,797 | Great Britain | Feb. 2, 1955  |

#### OTHER REFERENCES

The Journal of Chemical Physics, vol. 14, No. 1 (January 1946), pp. 1-7 relied on. (Copy in Div. 70.)